

stone : concrete.

Lime water and  
glycerin for hardening.

# UNITED STATES PATENT OFFICE.

CHARLES E. HALL AND ELMOR J. SALISBURY, OF CHICAGO, ILLINOIS.

## IMPROVEMENT IN ARTIFICIAL STONE.

Specification forming part of Letters Patent No. 157,511, dated December 8, 1874; application filed November 9, 1874.

*To all whom it may concern:*

Be it known that we, CHARLES E. HALL and ELMOR J. SALISBURY, of Chicago, Cook county, Illinois, have invented certain Improvements in a certain Compound called Artificial Stone, to be used in place of natural stone or brick, of which the following is a specification:

This invention relates to that class of compounds used in the construction of ornamental work, such as window and door caps, quoins, corbels, brackets, in fact all manner of architectural work; also, vases, urns, fountains, concrete walls, footings of buildings, &c.

To prepare this compound, take sixty-six (66) pounds of sand, thirty (30) pounds of hydraulic cement, four (4) pounds of baryta, making in all one hundred (100) pounds, to be moistened with a saturated solution of lime-water (not milk of lime) with the addition of four (4) ounces of glycerine to the gallon of water.

From this compound there can be some deviation, according to the class of work required.

The manner of working and mixing, also molding, is done in the same manner that all artificial stone is made.

The use of the baryta is to prevent the soda from working out on the surface. The glycerine with lime-water is used for hardening purposes.

We claim as our invention—

The compound as made from sand, gravel, and cement mixed with baryta, glycerine, and lime-water, substantially as and for the purpose hereinbefore set forth and shown.

CHARLES E. HALL.

ELMOR J. SALISBURY.

Witnesses:

GEORGE L. FORD,  
J. M. OSTROM.